

1

2,897,152

## LUBRICATING OILS

John Scotchford Elliott and Eric Descamp Edwards, London, England, assignors to C. C. Wakefield & Company Limited, London, England, a British company

No Drawing. Application March 4, 1957  
Serial No. 643,544

Claims priority, application Great Britain  
March 8, 1956

11 Claims. (Cl. 252—47.5)

This invention is for improvements in or relating to lubricating oils and is particularly concerned with lubricating oils which are to be used under conditions which tend to disrupt the lubricant film, which disruption more particularly takes place when the pressure between the bearing surfaces is very great. There have already been provided lubricants which have a high load-carrying capacity. Such lubricants are generally known in the trade as "extreme pressure" lubricants.

A large number of organic compounds have been proposed for use as extreme pressure agents, including various types of organic di- and polysulphides, and the corresponding derivatives of selenium. While the higher polysulphides are very effective in increasing the film rupture strength of the oil in which they are dissolved, they tend to be inherently unstable, corrosive, especially to copper and cuprous materials and to exert a pro oxidant effect on the oil. The disulphides, on the other hand, and other sulphur compounds containing relatively firmly-bound sulphur, though comparatively non-corrosive to copper, usually possess rather poor extreme pressure properties insufficient to warrant their use except in conjunction with other extreme pressure additives such as organic halogen compounds. Among this class of compounds there have been disclosed as additives for lubricating oils various simple alkyl and aryl thiocarbonates and thiocarbamates.

It is a nobject of the present invention to provide lubricating compositions having extreme pressure properties containing additives which are considerably less corrosive to copper and cuprous materials than many known extreme pressure agents of comparable load-carrying ability.

It is a further object of the invention to provide lubricating compositions having improved resistance to oxidation and foam-forming.

It is yet a further object of the invention to provide additives for turbine oils capable of increasing substantially their load-carrying capacity without at the same time increasing their tendency to oxidise or emulsify with water.

Thus at the present time many oils used for turbine lubrication consist of specially selected mineral oil blends stabilised against oxidation by the incorporation of antioxidant additives and containing also additives designed to protect ferrous metal parts against rusting or corrosion by, e.g. sea water. It is of course important that additional additives, incorporated in such oils for the purpose of enhancing their extreme pressure properties,

2

should not interfere in any way with the normal functions of the two foregoing classes of additive. Many turbine oils, especially marine turbine oils used by the Admiralty, are controlled as regards oxidation stability, salt water corrosion of ferrous metals, demulsification value and corrosive action on cuprous metals, by a very rigid specification. It is necessary, therefore, that extreme pressure additives incorporated therein should not adversely affect compliance with its clauses.

5 Many of the more commonly employed extreme pressure additives are detrimental in one or more respects. Thus chlorine compounds generally tend to promote oxidation and are also prone to hydrolysis with the subsequent liberation of hydrochloric acid which accelerates 10 rusting of ferrous metal parts.

Many sulphur compounds are also pro oxidant, and those which are without effect in this respect usually possess inadequate extreme pressure properties.

We have found a class of organic sulphur compounds 20 which possess surprisingly effective extreme pressure properties and which at the same time have valuable antioxidant properties and foam-inhibiting properties, which are relatively inactive towards copper and cuprous metals and which do not increase ferrous metal corrosion or 25 emulsification in the presence of water.

According to the present invention there is provided a lubricating composition comprising a mineral lubricating oil base and a minor proportion of a compound having the formula:



30 where  $R_1$  and  $R_2$  are alkyl, aryl, cycloalkyl radicals or 35 may together form part of a ring structure,  $R$  is  $CH_2$ ,



or



where  $R_4$  and  $R_5$  are hydrocarbon radicals, preferably  $CH_3$ , and  $R_3$  is an alkyl, aryl or cycloalkyl radical.

45 It is necessary to select  $R_1$ ,  $R_2$  and  $R_3$  so that the resulting product is oil-soluble in the proportions in which it is to be employed. Preferably  $R$  is  $CH_2$  and  $R_1$ ,  $R_2$  and  $R_3$  are alkyl radicals, the sum of the carbon atoms in  $R_1$ ,  $R_2$  and  $R_3$  being at least six.

50 If desired the radicals  $R_1$ ,  $R_2$  or  $R_3$  may contain halogen substituents, but when the additives are to be employed in turbine oils, the presence of halogen is to be avoided.

55 It would appear that the presence of ester groups situated in the alpha position to the dithiocarbamate group exerts an activating influence with the consequent production of extreme pressure properties substantially in excess of those obtainable by the use of the simple aliphatic or aromatic dithiocarbamates.

60 Examples of suitable compounds falling within the above formula include:

n-Butyl (dimethyl dithiocarbamyl) acetate,

n-Butyl (di-n-butyl dithiocarbamyl) acetate,

n-Butyl (di-isopropyl dithiocarbamyl) acetate,



Other esters prepared from the corresponding chloracetates and sodium dithiocarbamates included:

Ethyl (dimethyl dithiocarbamyl) acetate, crystalline solid, M.P. 61° C.

Isopropyl (dimethyl dithiocarbamyl) acetate, solid (percent S, 28.6; theoretical, 28.9%)

Isobutyl (dimethyl dithiocarbamyl) acetate, crystalline solid

Isopropyl (di-n-butyl dithiocarbamyl) acetate, low melting solid (percent N, 4.34; theoretical, 4.74)

n-Butyl (di-n-butyl dithiocarbamyl) acetate, light amber liquid (percent S, 20.3; theoretical, 20.1)

2-ethyl hexyl (cyclopentamethylene dithiocarbamyl) acetate, amber oil (percent S, 16.0; theoretical, 19.3)

Phenyl (di-n-butyl dithiocarbamyl) acetate, brown oil (percent S, 18.2; theoretical, 18.9)

n-Butyl  $\alpha$ (dimethyl dithiocarbamyl) isobutyrate (percent S, 21.8; theoretical, 24.3)

5

with a rubbing ratio of 3.4 to 1, loading being applied manually in increments of 5 lb. (scale reading) every 10 seconds until failure took place.

The additives were dissolved in a mineral oil blend such as "Oil B" which consisted of 80% of a solvent-refined mineral oil having a viscosity of about 150 seconds Redwood at 140° F. and 20% of a solvent-refined mineral oil having a viscosity of about 65 seconds Redwood at 140° F.

10 A very similar base oil, oil A, consisted of the two mineral oils described in Example 1 in 80:20 ratio. Oil A had a viscosity index of about 60 whereas oil B had a viscosity index of 95-100.

In certain blends marked with an asterisk an alkylated succinic acid type ferrous metal corrosion inhibitor was also present.

The results of load-carrying tests are summarized in Table 1.

TABLE 1

| Test No. | Base oil | Additives present                                                 | Percent sulphur provided by the additive | Four-ball machine tests         |                 |                    |         | SAE-SOD test failure load (lbs.) |  |
|----------|----------|-------------------------------------------------------------------|------------------------------------------|---------------------------------|-----------------|--------------------|---------|----------------------------------|--|
|          |          |                                                                   |                                          | Load, Kg., at incipient seizure | Weld point, Kg. | Mean wear (mms) at |         |                                  |  |
|          |          |                                                                   |                                          |                                 |                 | 100 Kg.            | 150 Kg. |                                  |  |
| 1        | A*       | None                                                              | Nil                                      | 32/36                           | 105             | 2.9                | -----   | 17 35                            |  |
| 2        | B*       | n-Butyl (dimethyl dithiocarbamyl) acetate (0.75%)                 | 0.20                                     | 95/100                          | 220             | 1.9                | 2.2     | 41 130                           |  |
| 3        | B*       | n-Butyl (dimethyl dithiocarbamyl) acetate (1.0%)                  | 0.26                                     | 95/100                          | 210             | 1.8                | 2.2     | 45 130                           |  |
| 4        | A        | n-Butyl (dimethyl dithiocarbamyl) acetate (1.5%)                  | 0.39                                     | 90/95                           | 190             | 1.4                | 2.0     | -----                            |  |
| 5        | A        | n-Butyl (di-n-butyl dithiocarbamyl) acetate (2.0%)                | 0.40                                     | 85/90                           | 200/220         | 1.9                | 2.1     | 110                              |  |
| 6        | B        | Isopropyl (di-n-butyl dithiocarbamyl) acetate (2.0%)              | 0.40                                     | 90/95                           | 230             | 1.7                | 2.0     | -----                            |  |
| 7        | B        | Phenyl (di-n-butyl dithiocarbamyl) acetate (2.15%)                | 0.40                                     | 110                             | 220             | 0.5                | 2.0     | 120                              |  |
| 8        | B        | 2-ethyl hexyl (cyclopentamethylene dithiocarbamyl) acetate (2.5%) | 0.40                                     | 120                             | 250             | 0.5                | 2.0     | -----                            |  |
| 9        | B        | n-Butyl $\alpha$ (dimethyl dithiocarbamyl) isobutyrate (1.65%)    | 0.36                                     | 85/130                          | 260             | 0.6                | 1.8     | -----                            |  |
| 10       | B        | $\beta$ -Chloroethyl (di-n-butyl dithiocarbamyl) acetate (2.0%)   | 0.40                                     | 95/100                          | 230             | 0.7                | 1.8     | 140                              |  |
| 11       | B        | S-n-hexyl di-n-butyl dithiocarbamate (1.92%)                      | 0.40                                     | 75/80                           | 200             | 1.8                | 2.1     | -----                            |  |
| 12       | B*       | S-n-hexyl di-n-butyl dithiocarbamate (1.25%)                      | 0.26                                     | 75/80                           | 170             | 2.0                | 2.5     | 39 120                           |  |
| 13       | A        | Di-benzyl disulphide (1.0%)                                       | 0.26                                     | 60/70                           | 260             | 1.0                | 1.5     | 135                              |  |

In an attempt to prepare  $\beta$ -chloroethyl (di-n-butyl dithiocarbamyl) acetate from  $\beta$ -chloroethyl monochloracetate and sodium di-n-butyl dithiocarbamate, an amber oil was obtained containing 8.7% Cl (theoretical, 11.1%). This evidently consisted of a mixture of compounds, some of the terminal chlorine atoms having been replaced.

Of the foregoing compounds, the first three listed were not soluble to the extent of 1.0 percent in mineral oil blend A, as used in the majority of the tests herein described.

To demonstrate the effectiveness of the compounds used in the compositions of the present invention as extreme pressure agents, tests were carried out on the well known four-ball machine similar to that described by Boerlage in "Engineering," 13th July 1933, volume 136, page 46. This apparatus comprised four steel balls arranged in the form of a pyramid. The top ball was held in a chuck attached to a spindle rotating at approximately 1500 r.p.m. and pressed against the three bottom balls clamped in a stationary ball holder. The balls were immersed in the oil to be tested. Tests were normally run for one minute at a series of different loads, but in certain cases supplementary tests were carried out for a duration of ten seconds, the "Mean Hertz Load" being calculated by the standard procedure described in U.S. Federal Specification VV-L-791d Method 650.3 (1950).

Certain tests were also carried out on the well known Society of Automotive Engineers (S.A.E.) Testing Machine described by Neely in the "Journal of the Society of Automotive Engineers," volume 39, page 293 (1936), by a modified procedure known as the S.A.E.-S.O.D. test, described by McTurk in Wright Aeronautical Development Centre (W.A.D.C.) Technical Report 53-88, page 70, (1953), published by the U.S. Department of Commerce Office of Technical Services. In this test procedure, the S.A.E. machine was operated at 1000 r.p.m. 75

40 In Table 1 tests 2 to 10 summarize the load-carrying properties of a variety of lubricating oils prepared in accordance with the present invention, from which it will be seen that in all cases the load-carrying capacity of the base oil (test 1) is greatly increased by the presence of organic dithiocarbamyl acetates. Tests 11 and 12 give 45 comparative figures obtained with a simple conventional organic dithiocarbamate, while test 13 quotes similar figures for dibenzyl disulphide, a well known extreme pressure additive known to be among the most effective of the simple organic disulphides.

50 It will be seen by comparing tests 2, 3, 12 and 13 that n-butyl (dimethyl dithiocarbamyl) acetate, which is typical of the additives of the present invention, gave significantly better results on the four ball machine than both the conventional dithiocarbamates and dibenzyl disulphide, although the total amounts of added sulphur in the oils were identical in tests 3, 12 and 13 and less in test 2. In this connection it should be pointed out that the load at the point of incipient seizure and the mean 55 Hertz load are generally believed to be the most significant of the four ball machine test results quoted.

60 By comparing test 11 with tests 4 to 10 (all about 40% added S) it will again be seen that the simple thiocarbamate ester was inferior to the compounds of the present invention.

65 When used in turbine oils, the organic dithiocarbamyl acetates not only do not adversely affect the properties of such oils but confer valuable antioxidant and anti-foaming properties, thus rendering unnecessary the addition of specific antioxidant and anti-foaming additives. If special load-carrying properties are not required, quite small amounts of the dithiocarbamyl acetates are sufficient to confer a degree of oxidation and foaming stability.

TABLE 2

| Test No. | Additive                                                                          | Base oil | Acidity (milligrams KOH per gram) | Demulsification value | Oxidation test                              |                                       | Salt water corrosion test | Foaming test (75° F.) |                   |
|----------|-----------------------------------------------------------------------------------|----------|-----------------------------------|-----------------------|---------------------------------------------|---------------------------------------|---------------------------|-----------------------|-------------------|
|          |                                                                                   |          |                                   |                       | Acidity after oxidation (mgs. KOH per gram) | Demulsification value after oxidation |                           | Tend-ency (mils.)     | Stability (mils.) |
| 14       | None                                                                              | A*       | 0.06                              |                       | Failed, unless antioxidant present.         | No rusting                            | 400                       | Nil (8 mins.)         |                   |
| 15       | n-Butyl (dimethyl dithiocarbamyl) acetate (1.5%)                                  | A*       | 0.06                              |                       | 0.11                                        | do                                    | 10                        | Nil (10 secs.)        |                   |
| 16       | n-Butyl (dimethyl dithiocarbamyl) acetate (0.75%)                                 | B*       | 0.06                              |                       | 0.11                                        | do                                    | Nil                       | Nil                   |                   |
| 17       | n-Butyl (dimethyl dithiocarbamyl) acetate (0.1%)                                  | A*       | 0.06                              |                       | 0.22                                        | do                                    | 110                       | Nil (2 mins.)         |                   |
| 18       | n-Butyl (di-n-butyl dithiocarbamyl) acetate (2.0%)                                | A*       |                                   |                       | 0.08                                        | 240                                   | No rusting                | 30                    | Nil (1.5 mins.)   |
| 19       | n-Butyl (dimethyl dithiocarbamyl) acetate (1.0%), Benzothiazole disulphide (0.1%) | B*       | 0.08                              | 150                   | 0.17                                        | 600                                   | do                        | 400                   | Nil (6 mins.)     |
| 20       | As test 19+0.1% zinc di-n-butyl dithiocarbamate                                   | B*       | 0.22                              | 240                   | 0.11                                        | 360                                   | do                        |                       |                   |

Table 2 illustrates the effect of the additives on typical turbine oils containing rust inhibitors which, with the

temperatures, a selection of the results being given in Table 3.

TABLE 3

[Tests recorded in this table were 24 hours duration, the base oil used throughout being oil B\*]

| Test No. | Additives present                                    | Appearance of copper strips at— |                       |                                |                                                 |                                 |
|----------|------------------------------------------------------|---------------------------------|-----------------------|--------------------------------|-------------------------------------------------|---------------------------------|
|          |                                                      | 100° C.                         | 110° C.               | 120° C.                        | 130° C.                                         | 140° C.                         |
| 21       | n-Butyl (dimethyl dithiocarbamyl) acetate (0.75%)    | Light brown/peacock stain.      | Dark peacock/magenta. | Dark peacock brown; 10% black. | Dark brown-black patch.                         | Dark peacock, black at one end. |
| 22       | As test No. 21+0.1% benzothiazole disulphide.        |                                 |                       | Orange brown powdery deposit.  |                                                 |                                 |
| 23       | As test No. 22+0.1% zinc di-n-butyl dithiocarbamate. | Reddish brassy stain.           | Light golden brown.   | Patch of yellow deposit.       | Light peacock with powdery light brown deposit. | Powdery light brown deposit.    |

There was no stain of the copper during 3 hours at 100° C. by n-butyl (dimethyl dithiocarbamyl) acetate in concentrations up to at least 1.5% in the absence of copper deactivators.

addition of a suitable antioxidant, would comply with British Admiralty Specification O.M. 100.

In test 17 the foaming test was carried out using as base oil the higher viscosity component of oil A without rust inhibitors.

The methods employed for determining the various values quoted above were standard methods described in "Standard Methods for Testing Petroleum and its Products," and having the following references:

Acidity I.P. 1/53 Method A (page 12, 1943 edition)  
Demulsification value I.P. 19/51 (page 117, 1951 edition)  
Oxidation test I.P. 114/53 P (page 395, 1953 edition)  
Salt water corrosion test I.P. 135/51 (page 390, 1951 edition) (modified to comply with O.M. 100 specification)  
Foaming stability I.P. 146/55 T (page 266, 1956 edition) (sequence 1 only quoted in the above table)

It will be seen from Table 2 that dithiocarbamyl acetates function effectively as antioxidants even in quite low concentrations, thus enabling turbine oils to satisfy the oxidation requirements of O.M. 100 specification (0.20 mg. KOH per gram maximum after oxidation test) without the addition of any other oxidation inhibitors.

By comparing tests 15 to 17 and 19 with test 14, it will be seen that they also function effectively as inhibitors of foaming. In test 20, the presence of zinc di-n-butyl dithiocarbamate evidently interfered with this effect.

Other properties of the oils, such as acidity, demulsification value and salt-water corrosion resistance were unaffected by the addition of the dithiocarbamylacetates.

In order to determine the effect of the lubricating oils of the present invention on copper at various temperatures, a series of tests were carried out in which strips of clean electrolytic quality copper foil 2 inches long and  $\frac{1}{2}$  inch wide were immersed in the oils in test tubes and heated in an oven for various periods of time at different

From Table 3 it will be seen that n-butyl (dimethyl dithiocarbamyl) acetate, which is typical of the additives of the present invention, is very mild in its action towards copper at temperatures of the order of 100 to 110° C. such as are encountered in steam turbines. Further improvement, particularly at the higher temperatures, may be obtained by including benzothiazole disulphide or a combination of this compound with zinc di-n-butyl dithiocarbamate.

A turbine oil complying with British Admiralty Specification O.M. 100 and consisting of base oil B containing 1.0% n-butyl (dimethyl dithiocarbamyl) acetate together with rust inhibitors as in Example 1 and copper deactivators as in Example 4 was subjected to a test on the well known Institution of Automobile Engineers (I.A.E.) 3/4" Centres Gear Machine described by Mansion in the Journal of the Institute of Petroleum, volume 38, page 633 (1952). This machine was operated at 4000 r.p.m. using En. 34 gears, with an oil temperature of 70° C. The average failure load was 93 lbs., a typical O.M. 100 turbine oil without load-carrying additive failing at 29 lbs.

To illustrate the use of dithiocarbamyl acetates in extreme pressure lubricants suitable for hypoid gears, the composition of Example 3 was tested on the four ball machine (standard one minute run), the weld-point being 490-500 kg. and the mean wear scar diameter at 100, 200, 300 and 400 kg. load being respectively 0.5, 1.2, 1.7 and 2.3 mms.

A commercially available hypoid gear oil having approximately the same viscosity and complying with U.S. Army Specification MIL-L-2105 welded at 400 kg., the mean wear scar diameter at 100, 200 and 300 kg. load being respectively 0.4, 1.5 and 2.0 mms.

We claim:

1. A lubricating composition consisting essentially of a mineral lubricating oil base containing from 0.05

percent up to 10 percent by weight of a compound having the formula:



where X is selected from the group consisting of



$\text{R}_1$  and  $\text{R}_2$  being lower alkyl radicals, and an aliphatic hydrocarbon chain of five carbon atoms attached to the nitrogen atom so as to form a ring structure, R is selected from the group consisting of  $-\text{CH}_2-$ ,



and



where  $\text{R}_4$  and  $\text{R}_5$  are lower alkyl radicals, and  $\text{R}_3$  is selected from the group consisting of a phenyl radical and an alkyl radical containing no more than eight carbon atoms.

2. A lubricating composition consisting essentially of a mineral lubricating oil base containing from 0.05 percent up to 10 percent by weight of a compound having the formula:



where  $\text{R}_1$  and  $\text{R}_2$  are lower alkyl radicals, R is selected from the group consisting of  $-\text{CH}_2-$ ,  $\text{R}_4-\text{C}-\text{H}$  and  $\text{R}_4-\text{C}-\text{R}_5$ , where  $\text{R}_4$  and  $\text{R}_5$  are lower alkyl radicals, and  $\text{R}_3$  is selected from the group consisting of a phenyl radical and an alkyl radical containing no more than eight carbon atoms.

3. A lubricating composition consisting essentially of a mineral lubricating oil base containing from 0.05 percent up to 10 percent of a compound having the formula:



where X is an aliphatic hydrocarbon chain of five carbon atoms attached to the nitrogen atom so as to form a ring structure, R is selected from the group consisting of  $-\text{CH}_2-$ ,



and



where  $\text{R}_4$  and  $\text{R}_5$  are lower alkyl radicals, and  $\text{R}_3$  is selected from the group consisting of a phenyl radical and an alkyl radical containing no more than eight carbon atoms.

4. A lubricating composition as claimed in claim 1, wherein  $\text{R}_3$  contains halogen substituents.

5. A lubricating composition consisting essentially of a mineral lubricating oil base containing from 0.05 percent up to 2 percent by weight of n-butyl (dimethyl dithiocarbamyl) acetate.

6. A lubricating composition consisting essentially of

a mineral lubricating oil base containing from 0.05 to 0.5 percent by weight of a compound having the formula:



where  $\text{R}_1$  and  $\text{R}_2$  are lower alkyl radicals and  $\text{R}_3$  is an alkyl radical containing not more than eight carbon atoms.

7. A steam turbine oil consisting essentially of a mineral lubricating oil base containing from 0.5 to 2 percent by weight of a compound having the formula:



where X is selected from the group consisting of



$\text{R}_1$  and  $\text{R}_2$  being lower alkyl radicals, and an aliphatic hydrocarbon chain of five carbon atoms attached to the nitrogen atom so as to form a ring structure, R is selected from the group consisting of  $-\text{CH}_2-$ ,



and



where  $\text{R}_4$  and  $\text{R}_5$  are lower alkyl radicals, and  $\text{R}_3$  is selected from the group consisting of a phenyl radical and an alkyl radical containing no more than eight carbon atoms.

8. A steam turbine oil consisting essentially of a mineral lubricating oil base containing from 0.5 to 2 percent by weight of a compound having the formula:



where  $\text{R}_1$  and  $\text{R}_2$  are lower alkyl radicals and  $\text{R}_3$  is an alkyl radical containing no more than eight carbon atoms.

9. A steam turbine oil as claimed in claim 7, wherein there is included from 0.005 to 0.1 percent by weight of an anti-rusting additive selected from the group consisting of an acid ester of a long-chain monoester of a polyhydric alcohol, and an alkylated succinic acid.

10. A steam turbine oil as claimed in claim 7, wherein there is included from 0.01 to 0.5 percent by weight of a copper-staining inhibitor selected from the group consisting of 2-mercapto benzothiazole and a derivative thereof capable of homolytic dissociation into free radicals

60



11. A lubricating composition consisting essentially of a mineral lubricating oil base containing from 0.05 percent up to 10 percent by weight of a compound having the formula:



where X is selected from the group consisting of



70

11

$R_1$  and  $R_2$  being lower alkyl radicals, and an aliphatic hydrocarbon chain of five carbon atoms attached to the nitrogen atom so as to form a ring structure,  $R$  is selected from the group consisting of  $-\text{CH}_2-$ ,



and



12

where  $R_4$  and  $R_5$  are lower alkyl radicals, and  $R_3$  is selected from the group consisting of a phenyl radical and an alkyl radical containing no more than eight carbon atoms, and from 1 to 15 percent by weight of 5 a chlorinated paraffin wax.

## References Cited in the file of this patent

## UNITED STATES PATENTS

- 10 2,160,851 Faust ----- June 6, 1939  
 2,160,880 Loane ----- June 6, 1939